

May 3, 1932.

H. NEUHAUSS

1,856,851

SINTERING REFRactories FROM MOLTEN MAGNESITE OR OTHER MATERIALS

Filed Aug. 1, 1928



Inventor  
Heinrich Neuhauss,  
by *W. Steel Seaman*  
Attorney.

## UNITED STATES PATENT OFFICE

HEINRICH NEUHAUSS, OF DUSSELDORF, GERMANY, ASSIGNOR TO THE AJAX METAL COMPANY, OF PHILADELPHIA, PENNSYLVANIA, A CORPORATION OF PENNSYLVANIA

## SINTERING REFRACTORIES FROM MOLTEN MAGNESITE OR OTHER MATERIALS

Application filed August 1, 1928. Serial No. 296,803.

My invention relates to methods of sintering furnace linings and other like surfaces.

One purpose of my invention is to form the sintered surface which is to be actively

engaged by a furnace charge, for example, against a mould or pattern which is afterward to be removed or destroyed, permitting accurate predetermination of the finished shape and surface of the sintered product.

10 A further purpose is to lay that surface first which is to be actively engaged by the furnace charge, making it possible to obtain more perfect sintering and greater uniformity and smoothness and continuity of the active surface than would otherwise be the case.

15 A further purpose is to pre-form sintered products and remove them to the place of indicated use, as distinguished from sintering linings, etc., in place within the furnace, making it possible to perform the sintering operations under the most favorable conditions of position, space and equipment and to obtain better sintered products.

20 A further purpose is to perform the sintering operation in a specially prepared sintering furnace free from the limitations and difficulties of location of the place of use.

25 A further purpose is to protect a sintered product from cracking by reason of temperature changes by relief of the backing supporting the surface of use.

30 A further purpose is to provide a form about or within which products are sintered and which is firm enough to stand the pressure of the sintered product and maintain its shape and yet is yieldable enough to avoid injury to the product, interspersing material for this purpose which can be baked out or burned out.

35 A further purpose is to form a special backing for a sintered refractory.

40 Further purposes will appear in the specification and in the claims.

45 My drawings are intended to be largely diagrammatic, and for this reason have been distorted freely for the purpose of illustration and without any attempt to maintain a scale. They are intended to illustrate a few only of the forms and ways upon which

or in or by which my invention may be carried out, those shown being selected primarily from the standpoint of illustration of the invention.

Figure 1 is a transverse section showing 55 one construction by which a cylinder or crucible may be pre-formed by sintering.

Figure 2 is a section of Figure 1 on line 2-2.

Figure 3 is a longitudinal section showing 60 a finished crucible.

Figure 4 is a top plan view of a form within which a special brick may be sintered.

Figure 5 is a section of Figure 4 upon the line 5-5. 65

Figure 6 is a fragmentary transverse section corresponding generally to Figure 1, but showing a different means of making the mould resilient.

Figure 7 is a transverse section showing a 70 cylinder which has been fully sintered and which has been grooved to relieve from cracking.

Figure 8 is a section corresponding to Figure 7 but showing the grooves as filled in. 75

In the drawings similar numerals indicate like parts.

Sintering, per se, is old and it is also old to sinter linings in furnaces, using magnesite, or other refractory materials such as dolomite, with flux. However, this sintering has to be performed in the difficult conditions and surroundings of intended use, has laid the final surface which is to be exposed for use last, unevenly and irregularly in many cases, and has permitted no suitable provision against cracking of the surface due to temperature changes. 85

With increasing size and thickness of furnace walls, it becomes more and more important to supply sintered bricks or blocks capable of being used as other bricks or blocks are used and to furnish cylinders, crucibles and other containers, or parts of containers pre-formed and capable of manufacture under the most favorable circumstances. These may then be shipped to and installed in their intended places of use. In some cases it will also be desirable to provide a parting 90

layer between the sintered refractory and the mould.

My invention is intended to provide methods by which sintered products can be cheaply and effectively constructed and to secure a better and different product from the sintered product which is now available.

The main characteristic of my sintering is that, as distinguished from sintering in place 10 I pre-form a product or shape by sintering it upon or against a mould or pattern from which it is subsequently removed, or which is subsequently broken from it to free the sintered product.

15 No attempt has been made to show a complete list of such products or the ways in which my invention may be practiced. I have shown means for moving the product and mould during the sintering operation and 20 an operation intended to be effective upon a stationary product, to indicate that neither the movement nor the stationary character of the parts during operation is essential to the broader features of my invention, and 25 have shown a complete crucible and partly complete crucible (a cylinder only, lacking a bottom) and a brick for the purpose of indicating that the completeness or lack of completeness of the product as compared 30 with the final container also are not material in the broader aspects of my invention.

In Figures 1 to 3 I have shown my invention as applied to the making of a crucible 10, using a rotatable form or pattern 11 upon 25 which to sinter the crucible. I prefer to make the form or pattern out of a type of material which will stand the temperature without undue surface shrinkage and which will be sufficiently yielding and easily destroyed to avoid injury to the product during the sintering or in removal of the pattern.

Because it is desirable to perform the sintering within a furnace where the heat can be applied to the best advantage I have shown 45 one for illustration which is convenient but not essential. In it provision has also been made for ready introduction of the pattern into the furnace.

The top 12, one end 13, base 14 and side 50 walls 15 are shown as fixed and comprise a casing. The base 14 forms a track for anti-friction balls or rollers 16 upon which is supported the shell 17 of a movable carrier including a refractory floor and closing end 55 18.

The walls of the furnace are formed of any suitable refractory for which I find dolomite well adapted.

The pattern or mould is shown in Figure 1 60 as slotted parallel with the axis at 19 to increase resilience and compressibility.

Because it is the intention to move the form 11 during sintering and the movement required by the character of product illustrated 65 is rotatorial, the pattern is mounted upon

a rotatable shaft 20 turning in bearings 21. From this shaft the pattern or mould 11 is supported at intervals by any suitable rods 22.

The carrier can be rolled into position within the casing to completely close the casing, 70 using the refractory floor of the shell 17 as the bottom of the furnace and exposing the surface of the mould to the intense heat from electric arcs fed through electrodes 23 or 24.

An opening is provided at 25 covered at 75 25' for inspection and for insertion of sintering materials.

Electrodes are shown in position to heat the sides and ends respectively of the product being sintered.

80 The pattern and mould may be made of any suitable neutral material of which dolomite is a cheap example but for which graphite is more lasting. I mix it with tar or some similar ingredient which holds the dolomite together and will burn out during sintering or during the pre-heating before so that the mould may be destroyed easily after the sintering of the product has been completed.

85 When the tar-dolomite pattern is in place the furnace is preferably heated preliminarily by flame from an oil or gas burner 26, while the cylinder is turned from time to time, in order to burn out the tar before the sintering begins and to permit a more gradual heating up of the pattern than would take place if the higher temperature of the arc were applied locally at one side or end.

90 After the cylinder has been heated up by the oil or gas burner it may be further heated by the electric arcs.

95 When the pattern is warm enough its movement will be stopped in order that one part of it may be made quite hot. A sintering material such as magnesite or other refractory powder, with a little slag, iron oxide or other flux will then be spread on the hot place and the heating will be continued until the test shows that the magnesite has been sintered. New parts are heated progressively and new, 100 thin layers of the powdered refractory and flux are added about the circumference until a complete cylinder has been formed. The application of powdered refractory and flux and heating is progressively continued in layers about the cylinder. Each successive part and layer is fused into homogeneous engagement with its adjacent parts and layers at the sides and beneath it so that when the cylinder 105 is completed it will comprise a homogeneous mass of thoroughly joined fused refractory.

110 Where it is desired to facilitate parting from the pattern a thin parting layer may be used initially. Various materials are suitable for this purpose such as pure powdered refractory (i. e. lacking a flux) or graphite. Where graphite is used for the mould its material serves this purpose also.

115 If a cylinder only be desired the product will now be complete, but if it be desired to

apply a bottom, as contemplated in the illustration of Figures 1 to 3, this bottom may be applied by progressive applications of thin layers of refractory fused into position, 5 either after the cylinder has been formed or progressively along with the applications of the layers of the cylinder, the arcs 23 at the end of the pattern being used to perform the sintering end operations.

10 While I have taken a crucible as my example and have assumed that it has circular cross-section inside and outside, my method is suited to sinter refractories of all shapes. This apparatus or other apparatus providing 15 movement is suited to sinter fully products of different cross-section, provided:

(a) That the products do not differ too far from true cylinders or other shapes to which the movement has been suited for the heat of 20 the arcs to properly sinter both the nearer and farther parts of the surface during movement of the pattern, or

(b) That the arcs, or pattern, be laterally moved one toward or away from the other 25 at the different portions of the pattern so as to maintain the arcs at a suitable sintering distance at all times from the portion of the surface to which the sintered layer is being applied.

30 The percentage of slag or flux need not be great. Satisfactory percentages of different fluxes are well known. It is desirable to reduce the slag content as the sintering operation proceeds.

35 While I have illustrated rotary movement only for the pattern it is evident that my sintering method may be applied to form a sintered product upon a pattern movable according to any other law than that of rotation, the pattern being moved progressively 40 to bring the successive portions of the pattern which upon layers of magnesite and flux have been placed within proper sintering distance of the arcs:

45 After the operation has been completed the pattern and carrier are removed from the furnace and the pattern or mould is broken out of the crucible leaving the crucible complete and finished with its inner surface composed of the layer of sintered material which 50 was first laid. Because of this fact this inner layer may be more accurately shaped and better finished than the last laid layers, which would receive the charge if, as previously, 55 the sintering were done in place. My method also makes it possible to pre-form the sintered products at the shop or factory under the most advantageous conditions.

60 In the form shown in Figures 4 and 5 I show a mould 27 made of a neutral material such as dolomite-tar containing an opening 28 adapted to mould a brick or block or hearth or other shape, for use in building up a refractory lining. This is intended to represent a 65 fixed sintered product pre-formed in a mould

and adapted to form either the whole or a part of a refractory bed or lining. The brick, block, hearth, etc., may be formed within a furnace of the same character as that shown in Figure 1 by laying and sintering successively layers of powdered refractory mixed with flux until the product has been completed, after which it is removed from the mould, or the mould is removed from it, so that the product may be shaped for use. 70

The size of the brick shown is small enough so that it would not be necessary to shift it beneath the arcs for sintering successive layers and the entire area of the brick may be sintered at one time. It will not, therefore, be necessary for the operator to shift the mould longitudinally nor laterally but such movements would be required and can easily be provided for when the product is a large one. 80

Where the furnace refractories sintered are fairly large there is a tendency of the refractory product to crack in the outer surface of the refractory i. e. that farthest removed from the molten metal. I have found that this can be relieved greatly by grinding grooves in the refractory at intervals, as shown at 29. The surface tension is relieved by the grinding of these grooves and the grooves do not have to go far under the surface to relieve against cracking where there is some tendency to break. I prefer not to leave the grooves open but to fill them in with powdered magnesite which need not be sintered into position. 95

In the form shown in Figures 4 and 5 it is desirable also to heat up the mould with oil or gas burners, before the arcs are applied burning out a large part of the tar (where this is used) before arc heating for sintering upon or within the mould is begun. 100

It will be seen that my invention makes up sintered crucibles, cylinders, blocks, etc. free from the difficulties of surroundings and location present where the sintering is done in place, that the surface of the sintered material which is intended to be used may be very exactly predetermined by the contour and finish of the mould, without the necessity for care in this particular in the manufacture, that the surface intended to be used may be given a finish better than that which is left at the back of a sintered wall where the work is done in place, and that the mould may be moved as need occurs to easily and conveniently render the whole surface accessible to the greatest extent for the sintering operation. 110

Such language as has been used as is based upon the mould being inside of the sintered refractory is to be given a meaning to cover a reversal of these positions as the invention will sometimes be applied to sintering within a mould. 125

This invention makes it possible also al- 130

ternatively to provide other protection against cracking of the backing of the refractory at the face of the backing.

It is possible to an unusual degree to vary 5 the hardness of the sintered product by use of a different flux or by varying the percentage of flux used or by the use of mixed powdered refractories or a different powdered refractory for the final (backing) portion 10 of the sintered refractory which are tougher than those used for the face of the sintered product, or to sinter the outer layers less completely than the inner portion, so as to leave a tougher and less frangible outer 15 layer to protect the outer part of the surface against cracking.

As will be seen the protection against cracking by grooving is based upon the idea that the outer surface shall be relieved from 20 circumferential strain due to temperature changes; that the methods by variation of the composition and by difference in extent of sintering are based upon the ideas of toughening the outer layer and altering its 25 surface characteristics to stand the strain and to reduce the frangibility, rather than by increasing the strength to withstand the strain.

In view of my invention and disclosure 30 variations and modifications to meet individual whim or particular need will doubtless become evident to others skilled in the art, to obtain all or part of the benefits of my invention without copying the structure 35 shown, and I, therefore, claim all such in so far as they fall within the reasonable spirit and scope of my invention.

Having thus described my invention what I claim as new and desire to secure by Letters Patent is:

1. The method of forming and sintering a refractory for holding molten metals, which consists in forming and sintering first the surface of the refractory which is to receive 45 the molten metal and subsequently and successively forming and sintering the backing of the refractory.

2. The method of forming and sintering material to form a refractory for use to hold 50 molten metals, which consists in forming the surface portion of the refractory which is to receive the molten metal against a pattern or mould, sintering it against the pattern or mould and successively and progressively increasing 55 the thickness of the sintered product by forming successive layers outside of the previously sintered product and sintering these layers into homogeneous engagement with the product already sintered to 60 form a backing for the surface.

3. The method of forming and sintering refractories intended to hold molten metal, which consists in forming and sintering the refractory against a portion of a pattern or 65 mould, and in moving the pattern or mould

relatively with respect to the source of sintering heat as the layer of refractory is progressively extended to cover a larger part of the mould.

4. The method of forming and sintering objects upon a mould which consists in forming the mould in part of elements adapted to be destroyed by heat, in preliminarily heating the mould to destroy these elements and leaving a mould capable readily of being destroyed, in sintering successive layers of refractory upon or within the mould to form a sintered product engaging the mould and in destroying the mould already weakened by destruction of these elements to render the sintered product available.

5. The method of forming and sintering objects upon a mould and removing the mould which consists in providing a mould having parts adapted to be weakened by the application of heat, in supplying heat to weaken the mould, in sintering a refractory about the mould and in destroying the heat-weakened mould.

6. The method of protecting a sintered refractory from cracking of the backing which consists in sintering against the mould a refractory wall adapted to hold the molten metal, in sintering successive layers of the refractory upon that layer against the mould and in finally forming a layer of less completely sintered refractory about the product to form the outside of the backing of the refractory.

7. The method of protecting a refractory against injury by cracking of its backing, which consists in sintering against a pattern or mould a layer which is adapted to hold the metal and in sintering successive layers of refractory about this layer to form a backing for it, forming the final backing of a refractory which is tougher to withstand temperature changes than the refractory face.

8. The method of forming sintered refractories for holding molten metal, which consists in forming the sintered product, at a distance from the place of intended use, against a pattern or mold, sintering it in place against the pattern or mold, and successively and progressively increasing the thickness of the sintered product by forming successive layers outside of the previously sintered product, and sintering these layers into homogeneous engagement with the product already sintered to form a backing for the surface.

9. The method of protecting a sintered powdered refractory intended to support molten metal from cracking in the backing surface farthest from the molten metal, which consists in grooving the backing of the refractory at intervals to relieve the stress in the backing.

10. The method of protecting a sintered powdered refractory intended to support

molten metal, which consists in grooving the backing of the refractory at intervals to relieve the stress in the backing and in filling the grooves formed with powdered magnesite.

11. The method of sintering, which comprises forming a mould having an ingredient adapted to burn out, in heating the mould to burn out this ingredient and in sintering a product upon the mould after the ingredient adapted to be burned out has been removed.

HEINRICH NEUHAUSS.

18

20

25

30

35

40

45

50

55

60

65